

## UNITED STATES PATENT OFFICE

WILLIAM H. WOOD, OF SOUTH EUCLID, OHIO

## WOOD VENEER AND PROCESS OF PREPARING SAME

No Drawing. Application filed April 7, 1924, Serial No. 704,698. Renewed July 26, 1928.

This invention relates to the treatment of wood veneer whereby its shipment and storage is facilitated, its life increased, its application permitted to unseasoned bases, and the life of its products increased. By 5 "veneer" I denote thin plates, sheets, or strips of wood either in the free state or after incorporation in an article of manufacture. Such thin strips are widely 10 used in the manufacture of baskets of all shapes, sizes, and types, generally by weaving, wattling, or tying; for making crates, hampers and vegetable barrels by nailing to thin wooden supports; and for producing 15 furniture, house finish, doors, etc., by being glued to the surface of more massive lumber of cheaper grade.

The production, handling and shipment of 20 these thin strips and sheets of wood varies with the different uses, but is always difficult and expensive. In the making of baskets it is necessary to employ the strips in a pliable condition for which purpose the strips are customarily made at the point of use, since 25 only certain woods can be shipped and stored without losing that pliable nature, and these are not the best or cheapest woods for basket making. Accordingly each locality is obliged to make its own strips, the logs being generally 30 kept in a vat of hot water until the moment of their transfer to the veneer cutter, and the strips being delivered to the weavers with a minimum of delay after they are produced. Even if strips are shipped short distances 35 they must be resoaked before using. These considerations generally require basket factories to maintain expensive, complicated machinery even though the production of the baskets is essentially a hand industry requiring only a minimum of machinery.

Excepting for the difficulty of shipping these strips, the basket stock could equally well be produced at some central point where lumber is readily available and shipped about the 45 country as need requires, thus enabling baskets to be made by small concerns to meet local requirements which is particularly necessary in a case where the bulk is so great compared with the value of the product.

50 Furthermore, while such a basket exhibits

a high degree of strength when new, this strength rapidly decreases owing to the drying of the veneer which causes it to become brittle, for which reason the life of such a basket is very short.

I have discovered that it is possible, by 55 impregnating the pores of the veneer with certain osmotic salts, to produce a veneer which will not warp, check or split to any appreciable extent; which can be shipped 60 and stored without becoming brittle or losing its elasticity, which can be made into baskets, crates, hampers, and the like with substantially equal readiness after months 65 of storage as when fresh and which exhibits a greatly increased length of life when made into such baskets, crates, hampers, etc. Other benefits and advantages of my discovery will become apparent as the description 70 proceeds.

In the performance of my said invention I impregnate the veneer with a water-soluble crystalline osmotic salt which crystallizes with sufficient water of crystallization to retain a sufficient amount of potential dampness to 75 prevent over-desiccation of the woody fibers without at the same time producing sensible dampness. This impregnation may occur either before or after cutting of the veneer; and the compound which I prefer to use for 80 this purpose is magnesium sulphate, commonly known as Epsom salt, dissolved in water to the extent of a hot concentrated solution. This salt crystallizes with seven molecules of water in accordance with the 85 formula  $MgSO_4 \cdot 7H_2O$ , the water of crystallization being so loosely held as largely to be driven off at the boiling point of water. It is very much more soluble in hot water than in cold water and exhibits high osmotic 90 pressure thereby penetrating readily into all parts of the lumber. It is not hygroscopic and does not become damp even in moist climates. By soaking the logs or strips in a hot concentrated solution, the same will be 95 found sensibly dry immediately upon cooling and without waiting for evaporation, the pores of the lumber being filled with crystalline Epsom salts which physically supports them against collapsing as well as preventing 100

overdrying of the cell walls. The shrinkage of such a veneer strip is markedly less than that of an untreated strip and its life is indefinitely prolonged. Basket stock can be shipped and stored indefinitely, and can be worked either wet or dry; although the soaking unless effected in a solution of the same composition, removes the crystals and leaves the veneer in condition for early disintegration the same as though it had never been treated. However, its flexibility is sufficiently great to permit its manipulation in the usual manner even while dry, in which case the benefits of the treatment are preserved to the resulting product.

Inasmuch as this veneer is intended primarily for food containers it is necessary that the salt employed for impregnating the same be non-poisonous; to prevent the strips sweating in moist weather it is necessary that the salt be non-hygroscopic; to prevent injury to the strips or food it is necessary that the material be non-alkaline.

However, I do not limit myself to magnesium sulphate for the purpose as certain other sulphate salts which crystallize with water of crystallization can be employed, such as sodium sulphate ( $Na_2SO_4 \cdot 10H_2O$ ), sodium thiosulphate ( $Na_2S_2O_3 \cdot 5H_2O$ ), aluminum sulphate ( $Al_2(SO_4)_3 \cdot 18H_2O$ ) and certain of the alums. Accordingly I do not limit myself except as set forth in my several claims hereto annexed.

Having thus described by invention what I claim is:

1. A wood veneer consisting of a sheet of porous wood impregnated with a water soluble substance consisting predominantly of free magnesium sulphate.
2. The process of preparing wood veneer for storage, shipment, and use which contains the step of soaking the same in a hot concentrated solution of a water soluble substance consisting predominantly of free magnesium sulphate.
3. Veneer for food-containers consisting of thin, pliable wood strips impregnated with a water soluble sulphate salt which crystallizes with water of crystallization, such as sodium sulphate, sodium-thio sulphate, aluminum sulphate, magnesium sulphate and alum.

In testimony whereof, I hereunto affix my signature.

WILLIAM H. WOOD.